

## UNITED STATES PATENT OFFICE

2,340,968

COMPOSITION CONTAINING MODIFIED  
WAXEugene Lieber, West New Brighton, Staten Island,  
N. Y., assignor to Standard Oil Development  
Company, a corporation of DelawareNo Drawing. Application November 1, 1939,  
Serial No. 302,320

13 Claims. (Cl. 252—59)

This invention relates to improved compositions containing a hydrocarbon wax and containing a wax-modifying agent and more particularly to such a wax-modifying agent when used as a pour depressor in lubricating oils, as well as to an improved method of preparing such wax-modifying agents.

Broadly, the invention comprises polymerizing halogeno alkyl aromatic hydrocarbons under controlled conditions to produce a light to viscous oil, recovering from said product a high molecular weight residue by distillation, preferably with fire and steam, and incorporating the resultant oil-soluble residue, which is found to have surprising wax-modifying properties, into a composition containing a hydrocarbon wax. The raw material to be polymerized may be a compound having the following general formula

RR'X

in which R is selected from the group consisting of aromatic hydrocarbons and halogen derivatives thereof, R' is a saturated aliphatic hydrocarbon group containing not more than 10 carbon atoms, preferably 3-10, and X represents one or more halogen atoms in the aliphatic group R'.

In carrying out the invention, it is preferred to use a halogenated alkyl aromatic hydrocarbon in which the aromatic part consists of one or two aromatic nuclei as in benzene and naphthalene. As to the halogen, it is believed that the best results are obtainable when the amount of halogen present in the alkyl group corresponds to one atom of halogen to one mol of alkyl aromatics. If such compounds are not readily available, they may be prepared by halogenating the alkyl aromatic hydrocarbon under conditions tending to produce chlorination only in the alkyl group rather than on the aromatic nucleus. In carrying out the halogenation, it is preferred to use chlorine because it is both effective and readily available at low cost. However, if desired, other halogens may be employed, such as bromine, iodine or fluorine. Generally, this chlorination should be carried out until about 5 to 25% of chlorine has been combined into the alkyl group of the alkyl aromatic compounds. In practice, it is found that chlorination to a content of 7 to 12% of chlorine gives results which are substantially superior to those obtainable with other chlorine contents. After the chlorination of the alkyl aromatic compound has been completed, the product is refined in such a way as to recover all of the compounds in which the halogen is incorporated essentially in the alkyl group. If

desired, this product, which will usually consist of a mixture of specific compounds in which chlorine atoms are attached to various carbon atoms of the alkyl group, may be subjected to some fractionation treatment such as distillation, precipitation, etc., in order to recover separately any one or more of the compounds.

In carrying out the polymerization step, a Friedel-Crafts type catalyst is used, preferably aluminum chloride, and this should be preferably anhydrous. Other catalysts of this type include ferric chloride, boron fluoride, zinc chloride, titanium tetrachloride and the like. The reaction involved here is called polymerization because there is only a single reactant, namely, the halogeno alkyl aromatic hydrocarbon compound. However, it is believed that the reaction actually involves some condensation to the extent that at least part of the chlorine incorporated in the side chains of the alkyl aromatic compounds combine with a hydrogen atom of an adjacent molecule and the two are liberated together as hydrogen chloride. Usually about 1 to 20% of aluminum chloride is used but preferably the amount should be between the narrower limits of about 5% to 15% but surprisingly superior results are obtained by using 10% and therefore this particular amount is preferred.

During the polymerization, it is preferred to use an inert solvent or diluent, which should preferably be present in an amount corresponding to somewhere between about 50% and 500% of the weight of the halogeno alkyl aromatic hydrocarbons to be polymerized. The reaction which usually proceeds vigorously is permitted to go at room temperature until it begins to slow down and then the reaction liquid is raised to a sufficient temperature to insure completion of the reaction, for instance, to 150° F., 200° F., or even 250° F. or higher, 150°-250° F. being preferred.

When the reaction is completed, the reaction mixture is cooled and then diluted with a further quantity of inert diluent and then the residual catalyst is inactivated by neutralizing with a mixture of water and alcohol. After removal of the aqueous layer by settling, centrifuging or other suitable means, the upper or kerosene layer is distilled to remove low-boiling products, and to leave a residue which is usually a resinous mass, which is the wax-modifying agent of this invention.

This product has been found particularly suitable as a pour depressor, i. e., a material which depresses or lowers the pour point of a lubricating oil (which is artificially determined at 5° F.

above the temperature at which the oil becomes solid). For instance, as shown in the data later, the addition of a small amount such as 2% of this wax modifier, will lower the pour point of an oil which normally has a pour point at 30° F. down to 5° F. or even far below 0° F. such as -25° F., the potency of the product being dependent upon the specific conditions used in the polymerization. When used as an addition agent to lubricating oil, the product of this invention has additional advantages such as that of imparting a greenish bloom and a deep red through color characteristic of Pennsylvania type oils.

Although it is primarily intended to use this wax modifier as a pour depressor in lubricating oils, it is also useful as an aid for settling, filtering or centrifuging a wax such as from a solution of hydrocarbon wax and an oil in a diluent such as naphtha, as used in dewaxing processes. For such a purpose, about 1% to 5% of the wax modifier is used, based upon the estimated amount of wax which is to be separated from the lubricating oil.

The wax modifier of this invention is also suitable for improving the texture of wax, such as paraffin wax to be used for coating paper, etc., in which case the amount of wax modifier to be used should usually be within the range of about 1% to 30% in the total composition of wax and wax modifier, preferably between the narrower limits of about 5% to 10%.

As examples of alkyl aromatic compounds which can be used as starting materials for the chlorination, the following may serve as representative:

|                 |                              |
|-----------------|------------------------------|
| Propyl benzene  | $C_6H_5 \cdot C_3H_7$        |
| Butyl benzene   | $C_6H_5 \cdot C_4H_9$        |
| Amyl benzene    | $C_6H_5 \cdot C_5H_{11}$     |
| Octyl benzene   | $C_6H_5 \cdot C_8H_{17}$     |
| Di-amyl benzene | $C_6H_5 \cdot (C_5H_{11})_2$ |

Instead of using plain alkyl aromatic compounds, one may also use halogen-substituted derivatives thereof, e. g., chlorinated compounds such as di-chlor amyl benzene having the formula  $C_6H_5(Cl)_2 \cdot C_5H_{11}$ . Also, instead of plain aromatic compounds with a single aromatic nucleus, di- or even poly-nuclear compounds may be used such as alpha- or beta-butyl naphthalene, alpha-amyl naphthalene, di-amyl naphthalene, etc. Furthermore, although the alkyl aromatic compounds and their substituted derivatives, as mentioned above, are preferred, chiefly due to the ease in directing their chlorination into the side chain, it is also possible to use mixtures containing same such as a refined fresh kerosene of high aromatic (about 30-35%) content which has been treated with aluminum chloride or other active chemical agents to remove undesirable constituents.

The invention will be better understood from the following data containing the test results reported in Table 1. The procedure used will first be explained as applicable to all the tests, unless otherwise specified.

A suitable refined alkylated aromatic compound, such as mono-amyl naphthalene, was chlorinated by passing chlorine through the hydrocarbon, maintained at about 200° to 225° F. The chlorination proceeded readily at this temperature to give a light-colored product and was continued until about 15% by weight of chlorine had been absorbed. 170 grams of the resulting chloro-amyl naphthalene were dissolved in 150 cc. of kerosene (made inert by treating with alu-

minum chloride prior to use) and 8.5 grams of aluminum chloride were added thereto while agitating at room temperature. The reaction proceeded readily as evidenced by the vigorous evolution of hydrogen chloride gas. After the addition of the aluminum chloride, the reaction temperature was raised to 220° F. and maintained thereafter for 60 minutes. The reaction mixture was then cooled and was diluted with a further quantity of refined kerosene (500 cc.) and was neutralized with a mixture of water and alcohol. After settling and removal of the lower aqueous layer, the upper or kerosene extract was distilled with fire and steam to 600° F. in order to remove low-boiling products. 120 grams of a dark green resinous mass was obtained as a bottom residue, which is the wax modifier of the present invention. To test the pour depressor characteristics of this material, a small amount, such as 2% or 5%, is dissolved in a lubricating oil having a known pour point, such as 30° F. (This is a pour point characteristic of a good grade Pennsylvania type oil after the usual dewaxing.)

Table 1

|    | Raw material          |      | AlCl <sub>3</sub> | Yield <sup>1</sup> | Pour pt., ° F., amt. pour depressor |          |
|----|-----------------------|------|-------------------|--------------------|-------------------------------------|----------|
|    | Name                  | Cl   |                   |                    | 2%                                  | 5%       |
| 35 | 1 Cl-amyl naphthalene | 15   | Per cent          | Per cent           | Per cent                            | Per cent |
| 2  | do                    | 15   | 5                 | 10                 | 69                                  | 0        |
| 3  | do                    | 15   | 10                | 20                 | 49                                  | -10      |
| 4  | do                    | 23   | 5                 | 5                  | 54                                  | 0        |
| 5  | do                    | 9.1  | 10                | 10                 | 22                                  | -25      |
| 6  | do                    | 9.1  | 15                | 15                 | 51                                  | -10      |
| 7  | Cl-amyl benzene       | 18.9 | 10                | 10                 | 27                                  | -10      |
| 8  | do                    | 9.3  | 10                | 10                 | 18                                  | -25      |
| 9  | do                    | 9.3  | 15                | 15                 | 35                                  | -5       |
| 40 | 10 Cl'd kerosene      | 22   | 5                 | 5                  | 27                                  | -10      |
|    |                       |      |                   |                    |                                     |          |

<sup>1</sup> Based on weight of chlorinated aromatic raw material used.

<sup>2</sup> The lube oil base stock used in making the pour point tests had a pour point of +30° F.

The product of test #1 when blended in a pale lubricating oil, imparted a greenish bloom and a deep red through color to it which is characteristic of Pennsylvania type oils. In test #1 the product was a dark green resinous mass. The product of test #2 had a similar appearance. In test #3 tetrachlorethane was used as solvent instead of kerosene and the 34 grams of anhydrous AlCl<sub>3</sub> were added slowly over a period of 60 minutes with suitable agitation and maintaining the reaction temperature at 68° F. then the reaction temperature was increased to 212° F. and maintained thereafter for 60 minutes. The product of test #3 when added to pale lubricating oil even at concentrations below 0.5% was found to impart a pleasing green bloom and fluorescence as well as a deep through red color to the oil. The product of test #3 was a dark brown resinous mass. The product of test #4 was a black resinous substance, which was found to be a powerful lubricating oil dye for pale oils. The product of test #5 was a black resinous substance. The product of test #7 was a black resinous substance which was also found to impart a greenish fluorescence and deep red through color to pale oils. The product of test #8 was also a black resinous material. In test #10 a kerosene fraction of petroleum was used which had an aniline point of 95° F. and the product obtained was a dark green resinous substance.

In the appended claims, the word "alkyl" is intended to mean a saturated aliphatic hydrocarbon group.

It is not intended that this invention be limited by any theory suggested as to the mechanism of the operation of the invention nor by any of the specific examples which have been given only for the sake of illustration, but only by the appended claims in which it is intended to claim all novelty inherent in the invention as broadly as the prior art permits.

I claim:

1. A composition comprising a hydrocarbon wax and an oil-soluble wax-modifying agent comprising an auto-condensation product of a compound having the following general formula: RR'X, in which R is a compound selected from the group consisting of aromatic hydrocarbons and halogen derivatives thereof, R' is a saturated aliphatic hydrocarbon group containing less than 10 carbon atoms, and X represents one or more halogen atoms in the aliphatic group R'.

2. A composition according to claim 1 in which the wax modifier is a residue obtained by fire and steam distillation to 600° F.

3. A composition according to claim 1 in which the wax modifier is an auto-condensation product of a chlor-alkyl naphthalene.

4. A composition according to claim 1 in which the wax modifier is an auto-condensation product of a chlor-alkyl benzene.

5. A composition comprising a hydrocarbon wax and a wax-modifying agent consisting essentially of an auto-condensation product of a chlor-  
amyl derivative of an aromatic hydrocarbon having less than 3 nuclei.

6. A lubricant comprising an oil containing dissolved waxy constituents which normally tend to prevent pouring of the oil at low temperatures, and also containing a small amount of a pour depressor comprising essentially an auto-condensation product of a halogen alkyl cyclic hydrocarbon having not more than 10 alkyl carbon atoms.

7. The method of preparing improved wax-containing compositions which comprises subjecting to auto-condensation a halogeno alkyl cyclic hydrocarbon having not more than 10 alkyl carbon atoms with a Friedel-Crafts catalyst under conditions to make a product of light to viscous oil consistency, separating from said product a wax modifier residue obtainable by fire and steam distillation to about 600° F., and incorporating said

wax modifier into a composition comprising a hydrocarbon wax.

8. The method of preparing improved wax-containing compositions which comprises chlorinating an alkylated cyclic hydrocarbon having not more than 10 alkyl carbon atoms to about 5% to 25% chlorine essentially in the alkyl group and subjecting to auto-condensation the resultant chlorinated hydrocarbon with about 1% to 20% of a Friedel-Crafts catalyst to make a product of light to viscous oil consistency, separating from said product a wax modifier residue and incorporating said wax modifier into a composition comprising a wax-containing lubricant.

15 9. Method according to claim 8 in which an alkylated aromatic hydrocarbon is chlorinated to about 7% to 12% chlorine and the resultant chlorinated alkylated aromatic hydrocarbon is subjected to auto-condensation with about 5% to 20 15% of aluminum chloride at room temperature until the reaction begins to slow down and then raising the temperature to about 150°-250° F. for about an hour.

10. Method according to claim 8 in which an amyl derivative of an aromatic hydrocarbon having less than 3 nuclei is chlorinated to about 9% chlorine and the resultant chlor-amyl aromatic compound is subjected to auto-condensation with about 10% of aluminum chloride.

30 11. The method of making lubricants which comprises chlorinating an alkylated cyclic hydrocarbon having not more than 10 alkyl carbon atoms to about 5% to 25% chlorine essentially in the alkyl group and polymerizing the resultant 35 chlorinated hydrocarbon with about 1% to 20% of a Friedel-Crafts catalyst to make a product of light to viscous oil consistency, separating from said product a wax modifier residue and incorporating said wax modifier into a composition comprising a wax-containing lubricant.

12. A lubricant comprising a major proportion of a waxy mineral lubricating oil containing dissolved therein a small amount of a pour depressor consisting of a product substantially non-volatile 45 up to about 600° F. under fire and steam distillation and obtained by the Friedel-Crafts auto-condensation of a chlorinated alkyl aromatic hydrocarbon containing about 5% to 25% of chlorine and having not more than 10 alkyl carbon atoms.

50 13. Lubricant according to claim 12, in which the pour depressor is derived by auto-condensation of chlorinated amyl benzene.

EUGENE LIEBER.